

# UNITED STATES PATENT OFFICE.

VASILI LIZOUNOFF, OF PITTSBURGH, PENNSYLVANIA, ASSIGNOR TO MARTIN A. ROSANOFF, OF PITTSBURGH, PENNSYLVANIA.

## OPERATION OF BLAST-FURNACES.

1,400,963.

Specification of Letters Patent. Patented Dec. 20, 1921.

No Drawing.

Application filed April 27, 1920. Serial No. 377,105.

To all whom it may concern:

Be it known that I, VASILI LIZOUNOFF, residing at Pittsburgh, in the county of Allegheny and State of Pennsylvania, a subject 5 of the Russian Empire, have invented or discovered certain new and useful Improvements in the Operation of Blast-Furnaces, of which improvements the following is a specification.

10 My invention relates to improvements in the operation of blast furnaces. It is common practice, in blast furnace operation, when a furnace is approaching the end of its life (which normally is about five years), 15 to devote it to the production of special iron alloys—ferro-manganese, for example, ferro-silicon, etc. It is to blast-furnace operation for such special uses that my invention particularly relates. It will of course be understood 20 that such special operation is not necessarily conditioned on nor consequent upon a prior normal use of the furnace through several years, but such is the usual and economically desirable practice.

25 Iron with a silicon content of 1 to 3.25% has wide use in the industries, and it is a matter of value and importance to produce it as cheaply as possible. The attempt so to regulate the blast-furnace operation as to 30 attain a product of precisely regulated composition is attended with considerable difficulty, so that the blast furnace cannot be looked to as the unaided and immediate source of iron silicon alloy for industrial use.

35 There is need of a supplementary operation, in which the uncertain proportions of the component metals may be brought certainly to the desired values. This supplementary operation is ordinarily performed in the 30 cupola furnace of the foundry. Under present-day practice the foundryman who proposes to produce iron silicon alloy of the quality called for in the industries, buys pig-iron having a smaller silicon content than 45 is required, and on the other hand he buys a ferro-silicon, and he compounds the two in his cupola furnace, proportioning his charge to afford him the desired composition of product. The foundryman's demand for a 50 ferro-silicon of high silicon content is therefore apparent.

In addition, ferro-silicon of high silicon content is required by steel mills, for producing steel castings for special purposes; and, finally, such high-silicon alloy is called 55 for by operators of Bessemer converters. Silicon has a high heat of combustion, and the Bessemer operator finds it a valuable ingredient, on occasion, of his converter charge; for, in being consumed under the 60 air blast, it becomes a most effective heating agent, and in consequence of its use the time of the run of a converter may be reduced.

At the present time the ferro-silicon of 65 high silicon content so required by foundryman, steel maker, operator of Bessemer converters, and others is produced in part in the blast furnace, in part in the electric furnace. Production in the electric furnace is relatively expensive, but in the electric-70 furnace operation there is no limitation on the proportion of the silicon ingredient attainable, whereas in the blast furnace under present-day conditions ferro-silicon production is limited to a product in which the 75 silicon ingredient is scarcely greater than 12%. The richer the ferro-silicon be in its silicon content the greater the price it can command.

By following my present invention, it becomes possible to produce in the blast furnace ferro-silicon in which the proportion of the silicon ingredient may be increased to as much as 25%.

In the operation now commonly pursued 85 in making ferro-silicon in the blast furnace the charge is made up of the following ingredients having the characteristics noted:—

The ore used is highly reducible (that is to say iron is present in the form of  $Fe_2O_3$ , 90 rather than in the form of  $Fe_3O_4$ ); furthermore, the ore chosen is lean, high in aluminum content, and also contains a certain amount of silica.

The limestone used is of a grade low in 95 magnesium and rich in calcium, and this for the reason that the magnesium present tends to increase the fluidity of the slag and to prevent in corresponding degree the formation of an iron alloy rich in silicon. The 100 limestone component of the charge is relatively small.

The coke used is low in sulfur. This particularity is consequent upon the fact that but little limestone is used, and therefore less sulfur can be carried off in the slag.

- 5 In addition to these, the major components of the charge, the following items should be noted: Quartz is generally added, for the purpose of increasing the silicon content of the burden; broken brick may be 10 added, to increase both the silicon and the aluminum contents; for the same purpose, clay may be added; and, finally, and again for the same purpose, various slags, waste products of iron and steel manufacture, are 15 sometimes thrown in as auxiliary materials.

The total silicon content of the furnace charge is about four or five times that which remains in the product.

In operation, the temperature of the air 20 blast is kept high and the furnace is driven slowly. In consequence, the output per unit of time is about one third of the output of the normal blast-furnace operation, when making cast iron.

25 I have so minutely described the practice hitherto of making ferro-silicon in the blast furnace, in order to bring into comparison with it my own practice and to emphasize the features of novelty.

30 My improved procedure also is preferably (not necessarily, of course) carried out in a blast furnace which is approaching the end of its term of life.

According to my invention, the furnace 35 charge is far different from that hitherto employed to produce ferro-silicon. I preferably use no ore, nor do I ordinarily use any limestone, or quartz, brick, or clay. In place of ore, I preferably use heating-furnace cinder and rely on it primarily as the 40 source of iron (and of silicon as well). This heating-furnace cinder is a familiar by-product of heating-furnaces used in steel mills and wherever steel is fabricated, and 45 usually has approximately the following composition, given here as typical: iron, 44.20%; manganese, 1.30%; phosphorus .06%; sulfur, 4%; silica, 34.10%; alumina, 5.40%; calcium oxid, 4.20%; magnesium 50 oxid, 2.40%.

In place of limestone, I use blast-furnace slag, and this in especially large quantities. The normal, usual slag contains, essentially, 55 silica, 32%; alumina, 18%; and calcium oxid and magnesium oxid together, about 38%.

I use coke low in sulfur, as in the operation now commonly practised and characterized above, and I use somewhat more coke than that operation requires. The normal 60 blast furnace operation for making ordinary cast iron requires about .80 to 1.20 units of coke for every unit of iron produced; the old operation of producing ferro-silicon in the blast furnace characterized above re-

quires at least 1.70 units of coke per unit 65 of product; my improved operation which I now am describing, requires 1.75 to 2 units of coke to each unit of product. It must not, however, be supposed that my operation is therefore more costly than the old operation; to the contrary, considering the economies realized in other respects in the composition of the furnace charge, the advantage is emphatically in my favor.

These ingredients are so compounded that 75 the slag produced in my operation shall have this approximate percentage of the essential ingredients: silica, 38%; alumina, 19%; and calcium oxid and magnesium oxid together, 38%.

80 Some further notes on the ingredients of my furnace charge may be made: First, chemically, it is advantageous to derive the needed calcium from slag rather than from limestone—advantageous because the slag 85 substituted for limestone itself brings into the furnace charge excess measures of silicon, which of course are present during the operation, to manifest advantage in the chemical formation of the desired product. Another advantage lies in this, that blast-furnace slag is practically free from phosphorus, as limestone often is not. Of the blast-furnace slag, it is to be remarked that 90 it is now an almost valueless substance, and 95 is indeed an encumbrance upon ordinary blast-furnace operations.

It may finally be asked, whether the absence of limestone would not result in the introduction of excessive amounts of sulfur 100 into the ferro-silicon product. All my experience shows that this is not the case; about half of the sulfur is expelled at the high temperature of my operation, through volatilization, and half is carried off by the 105 excess of slag produced. The high temperature of operation here alluded to arises from the comparatively large amounts of fuel used, from the high heat of the blast which I employ, from the slow rate at which the 110 furnace is driven, and from the high melting point of the resulting slag.

115 The advantages of using heating-furnace cinder, rather than iron ore, are, first, that it costs relatively little; and second, that the silicon present in large quantities in this cinder, combined chemically as it is with FeO in the form of silicates of iron, now appears (and this is my discovery) to be in excellent condition, chemically, to make 120 new union, under the reducing conditions obtaining in the blast-furnace operation, with the iron alone, and so to form the desired ferro-silicon. The mere presence of both iron and silicon in the furnace charge, 125 each in combined state, and each in a separate combination, affords no assurance that in the operation of the furnace the silicon

will be released to unite with the iron. And, so far as concerns heating-furnace cinder, the belief has been that, inasmuch as it contains iron in the form of silicate, it is quite generally inappropriate as an iron-affording component of the blast-furnace charge, on account of the difficulty of reducing iron from silicates. My experience has led to the discovery that under the special conditions of ferro-silicon production, these ferro-silicates are reduced very readily; and in that they contain iron and silicon already chemically combined, they constitute the very best material from which to derive ferro-silicon.

As for the blast-furnace slag in the charge, it should, as has been said, be introduced in large quantities. If too little slag were used, the bottom of the furnace would soon rise; that is to say, a layer of congealed ferro-silicon would rapidly grow upon the bottom of the furnace. An excess of molten slag keeps the bottom of the furnace washed clean of any such accumulation. There follows this further benefit: the furnace may always be tapped through the iron notch, whereas, in ordinary practice it sometimes happens that, because of bottom incrustation, the molten ferro-silicon must be tapped through the cinder notch.

Still another advantage consequent upon the use of a large excess of blast-furnace slag lies in this: After the ferro-silicon is already formed, there is danger that some of the silicon may be burned out (this is a surface action, of course) by the gases present in the furnace. The great excess of slag affords a surface cover, and mechanically protects the new-formed molten ferro-silicon.

Having now described the furnace charge, I have still to explain the method by which the operation is brought into practice. The operation of my invention is brought into effect gradually. The furnace should have been in blast for several days before the modifications in operation are begun which, when completed, will constitute the ferro-silicon producing operation of my invention.

Let it be supposed, then, that a furnace is in blast, and is carrying the usual burden. When now the ferro-silicon process is to be introduced, the additions to the furnace charge are modified. As the burden goes down, the operator begins filling with a mixture of coke and blast furnace slag. When a layer of this mixture has been spread, the ensuing addition consists of the same mixture, but with a relatively small addition of heating-furnace cinder (about 40% of the ultimate and normal ratio). As further additions are made the ratio of cinder will be gradually increased, until at last it comes to normal.

While such adaptation is being made the

melt—the product of the furnace, which initially was ordinary pig iron—will begin to acquire an increasing silicon content. The melt will from time to time be tested, and the charging will be governed according to the results of such test. The increase of the ratio of heating-furnace cinder is so timed that the normal ratio is reached at a time when the silicon content in the product has reached a value of 18 to 20%.

From this point, the operation is straightforward.

It is advisable, as is common practice in blast-furnace operation, to prevent loss in the form of outblown dust by wetting the furnace charge at the top.

According to the old ferro-silicon process practised in the blast furnace and characterized above, a product is obtained in which the silicon content scarcely exceeds 12%. In the practice of my invention now described I double that figure and produce ferro-silicon with a silicon content of as much as 25%. For reasons stated, this is a far more valuable product.

The ferro-silicon operation is preferably practised upon a furnace which is approaching the end of its term of life. The old process of making ferro-silicon brings the life of the furnace to an end after about three to four months; in the practice of my invention the furnace will last four to five months—a gain of 30%.

In the ensuing claims I define the essence of my present invention. The features of operation, over and above what is so defined, and described above, are described in an exemplary way merely, and are not to be understood as limitations upon the invention. The invention will be practised if the features defined in the claims be present.

I claim as my invention:

1. The method herein described of producing ferro-silicon in a blast furnace which consists in conducting the blast-furnace operation upon a furnace charge composed of blast-furnace slag, coke, and heating-furnace cinder.
2. The method herein described of producing ferro-silicon in a blast furnace which consists in conducting the blast-furnace operation upon a furnace charge including heating-furnace cinder and a heat-affording substance.
3. The method herein described of producing ferro-silicon in a blast furnace which consists in modifying the charge of a continuously operating blast furnace and introducing a mixture of blast-furnace slag and coke with an increasing ingredient of iron in chemical combination.
4. The method herein described of producing ferro-silicon in a blast furnace which

consists in modifying the charge of a continuously operating blast furnace and introducing a mixture of blast-furnace slag and coke, with an increasing ingredient of 5 heating-furnace cinder.

5. The method herein described of producing ferro-silicon from an iron-silicate which consists in subjecting a body of iron-silicate in the presence of a heating agent

and fluxing material not having avidity for silicon to the reducing action of a blast furnace.

In testimony whereof I have hereunto set my hand.

VASILI LIZOUNOFF.

Witnesses:

BAYARD H. CHRISTY,  
MARTIN A. ROSANOFF.